



US009925424B2

(12) **United States Patent**  
**Ladd et al.**

(10) **Patent No.:** **US 9,925,424 B2**  
(45) **Date of Patent:** **\*Mar. 27, 2018**

(54) **GOLF BALL COMPOSITIONS**

(71) Applicant: **Acushnet Company**, Fairhaven, MA (US)

(72) Inventors: **Derek A. Ladd**, Acushnet, MA (US); **David A. Bulpett**, Boston, MA (US); **Scott Cooper**, Freetown, MA (US); **Michael J. Sullivan**, Old Lyme, CT (US)

(73) Assignee: **Acushnet Company**, Fairhaven, MA (US)

(\*) Notice: Subject to any disclaimer, the term of this patent is extended or adjusted under 35 U.S.C. 154(b) by 0 days.

This patent is subject to a terminal disclaimer.

(21) Appl. No.: **15/283,545**

(22) Filed: **Oct. 3, 2016**

(65) **Prior Publication Data**

US 2017/0021234 A1 Jan. 26, 2017

**Related U.S. Application Data**

(62) Division of application No. 13/723,529, filed on Dec. 21, 2012, now Pat. No. 9,457,236.

(51) **Int. Cl.**

**A63B 37/04** (2006.01)  
**A63B 37/00** (2006.01)

(52) **U.S. Cl.**

CPC ..... **A63B 37/0092** (2013.01); **A63B 37/0043** (2013.01); **A63B 37/0062** (2013.01); **A63B 37/0076** (2013.01); **A63B 37/0007** (2013.01); **A63B 37/0018** (2013.01)

(58) **Field of Classification Search**

USPC ..... 473/374, 367, 370, 377  
See application file for complete search history.

(56) **References Cited**

**U.S. PATENT DOCUMENTS**

|                   |         |                                        |
|-------------------|---------|----------------------------------------|
| 5,782,707 A       | 7/1998  | Yamagishi et al.                       |
| 6,679,791 B2      | 1/2004  | Watanabe                               |
| 7,731,606 B2 *    | 6/2010  | Sullivan ..... A63B 37/0003<br>473/376 |
| 2003/0073517 A1 * | 4/2003  | Ichikawa ..... A63B 37/0003<br>473/378 |
| 2010/0160086 A1 * | 6/2010  | Sullivan ..... A63B 37/0062<br>473/374 |
| 2010/0227707 A1 * | 9/2010  | Sullivan ..... A63B 37/0062<br>473/374 |
| 2010/0273577 A1 * | 10/2010 | Sullivan ..... A63B 37/0044<br>473/374 |
| 2010/0331117 A1 * | 12/2010 | Sullivan ..... A63B 37/0003<br>473/377 |
| 2011/0014999 A1 * | 1/2011  | Sullivan ..... A63B 37/0044<br>473/376 |
| 2011/0053709 A1 * | 3/2011  | Comeau ..... A63B 37/0003<br>473/376   |
| 2011/0159996 A1 * | 6/2011  | Sullivan ..... A63B 37/0003<br>473/373 |
| 2011/0224022 A1 * | 9/2011  | Sullivan ..... A63B 37/0003<br>473/376 |

(Continued)

*Primary Examiner* — Gene Kim

*Assistant Examiner* — Matthew B Stanczak

(74) *Attorney, Agent, or Firm* — Mandi B. Milbank

(57) **ABSTRACT**

Disclosed herein are multilayer golf balls having a layer with a higher Shore C hardness and a lower Shore D hardness than another layer.

**2 Claims, 1 Drawing Sheet**



(56)

**References Cited**

U.S. PATENT DOCUMENTS

2011/0287861 A1 \* 11/2011 Sullivan ..... A63B 37/0044  
473/376  
2012/0115635 A1 5/2012 Sullivan  
2012/0115640 A1 5/2012 Bulpett  
2012/0115643 A1 5/2012 Sullivan

\* cited by examiner



FIG. 1

## GOLF BALL COMPOSITIONS

## CROSS-REFERENCE TO RELATED APPLICATIONS

The present application is a division of U.S. patent application Ser. No. 13/723,529, filed Dec. 21, 2012, the entire disclosure of which is hereby incorporated herein by reference.

## FIELD OF THE INVENTION

The present invention relates generally to golf balls comprising a first layer having a higher Shore C hardness and a lower Shore D hardness than a second layer.

## BACKGROUND OF THE INVENTION

The relative hardnesses between two materials is usually the same regardless of the hardness scale. For example, if a first material has a higher Shore C than a second material, then the first material will typically have a higher Shore D than the second material. Thus, in conventional multilayer golf balls, if the Shore C hardness of the composition used to form a first layer is greater than that of the composition used to form a second layer, then the Shore D hardness of the first layer composition will also be greater than that of the second layer composition.

The present invention provides a novel golf ball construction wherein the typical relative hardness relationship does not exist between two of the layers. For example, if the composition used to form a first layer has a higher Shore C hardness than the composition used to form a second layer, then the composition used to form the first layer will have a lower Shore D hardness than the composition used to form the second layer.

## SUMMARY OF THE INVENTION

In one embodiment, the present invention is directed to a golf ball comprising a first layer formed from a first composition and a second layer formed from a second composition. The Shore C hardness of the first composition is greater than the Shore C hardness of the second composition, and the Shore D hardness of the first composition is less than the Shore D hardness of the second composition.

In another embodiment, the present invention is directed to a golf ball comprising a solid, single layer core, an inner cover layer, and an outer cover layer, the core having a higher Shore C hardness and a lower Shore D hardness than that of the inner cover layer.

In another embodiment, the present invention is directed to a golf ball comprising an inner core layer, an outer core layer, an inner cover layer, and an outer cover layer, the outer core layer having a higher Shore C hardness and a lower Shore D hardness than that of the inner cover layer.

In another embodiment, the present invention is directed to a golf ball comprising a solid, single layer core, an inner cover layer, and an outer cover layer, the core having a lower Shore C hardness and a higher Shore D hardness than that of the inner cover layer.

In another embodiment, the present invention is directed to a golf ball comprising an inner core layer, an outer core layer, an inner cover layer, and an outer cover layer, the outer core layer having a lower Shore C hardness and a higher Shore D hardness than that of the inner cover layer.

## BRIEF DESCRIPTION OF THE DRAWINGS

FIG. 1 is a cross-sectional view of a golf ball according to one embodiment of the present invention.

## DETAILED DESCRIPTION

FIG. 1 shows a golf ball 30 according to one embodiment of the present invention, including an inner core layer 32, an outer core layer 34, an inner cover layer 36, and an outer cover layer 38.

Golf balls of the present invention are multilayer balls (i.e., solid core of one or more layers and a cover of one or more layers), having a novel construction wherein one layer has a higher Shore C hardness and a lower Shore D hardness than that of another layer. Such hardness relationship can be achieved by forming the layers from the same material and adjusting the material's hardness to a first desirable level for one layer and a second desirable level for another layer (e.g., two polyurethane layers having different isocyanate levels), or by forming the layers from different materials (e.g., an ionomer layer and a rubber layer), wherein each material's hardness is adjusted to the desirable level. Thus, each layer of the ball is formed from a composition independently selected from the following thermoset and thermoplastic compositions, so long as the composition used to form one layer has a higher Shore C hardness and a lower Shore D hardness than the composition used to form another layer.

Suitable thermoset compositions include, but are not limited to, natural rubbers, polybutadienes, polyisoprenes, ethylene propylene rubbers (EPR), ethylene-propylene-diene rubbers (EPDM), styrene-butadiene rubbers, butyl rubbers, halobutyl rubbers, polyurethanes, polyureas, acrylonitrile butadiene rubbers, polychloroprenes, alkyl acrylate rubbers, chlorinated isoprene rubbers, acrylonitrile chlorinated isoprene rubbers, polyalkenamers, phenol formaldehydes, melamine formaldehydes, polyepoxides, polysiloxanes, polyesters, alkyds, polyisocyanurates, polycyanurates, polyacrylates, and combinations of two or more thereof.

Suitable initiator agents include organic peroxides, high energy radiation sources capable of generating free radicals, C—C initiators, and combinations thereof. High energy radiation sources capable of generating free radicals include, but are not limited to, electron beams, ultra-violet radiation, gamma radiation, X-ray radiation, infrared radiation, heat, and combinations thereof. Suitable organic peroxides include, but are not limited to, dicumyl peroxide; n-butyl-4,4-di(t-butylperoxy) valerate; 1,1-di(t-butylperoxy)3,3,5-trimethylcyclohexane; 2,5-dimethyl-2,5-di(t-butylperoxy) hexane; di-t-butyl peroxide; di-t-amyl peroxide; t-butyl peroxide; t-butyl cumyl peroxide; 2,5-dimethyl-2,5-di(t-butylperoxy)hexyne-3; di(2-t-butyl-peroxyisopropyl)benzene; dilauroyl peroxide; dibenzoyl peroxide; t-butyl hydroperoxide; lauryl peroxide; benzoyl peroxide; and combinations thereof. Examples of suitable commercially available peroxides include, but are not limited to Perkadox® BC dicumyl peroxide, commercially available from Akzo Nobel, and Varox® peroxides, such as Varox® ANS benzoyl peroxide and Varox® 231 1,1-di(t-butylperoxy)3,3,5-trimethylcyclohexane, commercially available from RT Vanderbilt Company, Inc. Peroxide initiator agents are generally present in the thermoset composition in an amount of at least 0.05 parts by weight per 100 parts of the base polymer, or an amount within the range having a lower limit of 0.05 parts or 0.1 parts or 0.8 parts or 1 part or 1.25 parts or 1.5 parts by weight per 100 parts of the base polymer, and an upper

limit of 2.5 parts or 3 parts or 5 parts or 6 parts or 10 parts or 15 parts by weight per 100 parts of the base polymer.

Coagents are commonly used with peroxides to increase the state of cure. Suitable coagents include, but are not limited to, metal salts of unsaturated carboxylic acids; unsaturated vinyl compounds and polyfunctional monomers (e.g., trimethylolpropane trimethacrylate); phenylene bismaleimide; and combinations thereof. Particular examples of suitable metal salts include, but are not limited to, one or more metal salts of acrylates, diacrylates, methacrylates, and dimethacrylates, wherein the metal is selected from magnesium, calcium, zinc, aluminum, lithium, nickel, and sodium. In a particular embodiment, the coagent is selected from zinc salts of acrylates, diacrylates, methacrylates, dimethacrylates, and mixtures thereof. In another particular embodiment, the coagent is zinc diacrylate. When the coagent is zinc diacrylate and/or zinc dimethacrylate, the coagent is typically included in the thermoset composition in an amount within the range having a lower limit of 1 or 5 or 10 or 15 or 19 or 20 parts by weight per 100 parts of the base polymer, and an upper limit of 24 or 25 or 30 or 35 or 40 or 45 or 50 or 60 parts by weight per 100 parts of the base polymer. When one or more less active coagents are used, such as zinc monomethacrylate and various liquid acrylates and methacrylates, the amount of less active coagent used may be the same as or higher than for zinc diacrylate and zinc dimethacrylate coagents.

The thermoset composition optionally includes a curing agent. Suitable curing agents include, but are not limited to, sulfur; N-oxydiethylene 2-benzothiazole sulfenamide; N,N-di-ortho-tolylguanidine; bismuth dimethyldithiocarbamate; N-cyclohexyl 2-benzothiazole sulfenamide; N,N-diphenylguanidine; 4-morpholinyl-2-benzothiazole disulfide; dipentamethylenethiuram hexasulfide; thiuram disulfides; mercaptobenzothiazoles; sulfenamides; dithiocarbamates; thiuram sulfides; guanidines; thioureas; xanthates; dithiophosphates; aldehyde-amines; dibenzothiazyl disulfide; tetraethylthiuram disulfide; tetrabutylthiuram disulfide; and combinations thereof.

The thermoset composition optionally contains one or more antioxidants. Antioxidants are compounds that can inhibit or prevent the oxidative degradation of the base polymer. Some antioxidants also act as free radical scavengers; thus, when antioxidants are included in the thermoset composition, the amount of initiator agent used may be as high or higher than the amounts disclosed herein. Suitable antioxidants include, for example, dihydroquinoline antioxidants, amine type antioxidants, and phenolic type antioxidants.

The thermoset composition optionally includes a soft and fast agent. Preferably, the thermoset composition contains from 0.05 phr to 10.0 phr of a soft and fast agent. In one embodiment, the soft and fast agent is present in an amount within a range having a lower limit of 0.05 or 0.1 or 0.2 or 0.5 phr and an upper limit of 1.0 or 2.0 or 3.0 or 5.0 phr. In another embodiment, the soft and fast agent is present in an amount of from 2.0 phr to 5.0 phr, or from 2.35 phr to 4.0 phr, or from 2.35 phr to 3.0 phr.

Suitable soft and fast agents include, but are not limited to, organosulfur and metal-containing organosulfur compounds; organic sulfur compounds, including mono, di, and polysulfides, thiol, and mercapto compounds; inorganic sulfide compounds; blends of an organosulfur compound and an inorganic sulfide compound; Group VIA compounds; substituted and unsubstituted aromatic organic compounds that do not contain sulfur or metal; aromatic organometallic compounds; hydroquinones; benzoquinones; quinhydrones;

catechols; resorcinols; and combinations thereof. In a particular embodiment, the soft and fast agent is selected from zinc pentachlorothiophenol, pentachlorothiophenol, ditolyl disulfide, diphenyl disulfide, dixylyl disulfide, 2-nitroresorcinol, and combinations thereof.

The thermoset composition may contain one or more fillers. Exemplary fillers include precipitated hydrated silica, clay, talc, asbestos, glass fibers, aramid fibers, mica, calcium metasilicate, zinc sulfate, barium sulfate, zinc sulfide, lithopone, silicates, silicon carbide, diatomaceous earth, carbonates (e.g., calcium carbonate, zinc carbonate, barium carbonate, and magnesium carbonate), metals (e.g., titanium, tungsten, aluminum, bismuth, nickel, molybdenum, iron, lead, copper, boron, cobalt, beryllium, zinc, and tin), metal alloys (e.g., steel, brass, bronze, boron carbide whiskers, and tungsten carbide whiskers), oxides (e.g., zinc oxide, tin oxide, iron oxide, calcium oxide, aluminum oxide, titanium dioxide, magnesium oxide, and zirconium oxide), particulate carbonaceous materials (e.g., graphite, carbon black, cotton flock, natural bitumen, cellulose flock, and leather fiber), microballoons (e.g., glass and ceramic), fly ash, core material that is ground and recycled, nanofillers and combinations thereof.

The thermoset composition may also contain one or more additives selected from processing aids, such as transpolyisoprene (e.g., TP-301 transpolyisoprene, commercially available from Kuraray Co., Ltd.) and transbutadiene rubber; processing oils; plasticizers; coloring agents; fluorescent agents; chemical blowing and foaming agents; defoaming agents; stabilizers; softening agents; impact modifiers; free radical scavengers; accelerators; scorch retarders; and the like.

Non-limiting examples of suitable commercially available thermoset rubbers are Buna CB high-cis neodymium-catalyzed polybutadiene rubbers, such as Buna CB 23, and Buna CB high-cis cobalt-catalyzed polybutadiene rubbers, such as Buna CB 1220 and 1221, commercially available from Lanxess Corporation; SE BR-1220, commercially available from The Dow Chemical Company; Europrene® NEOCIS® BR 40 and BR 60, commercially available from Polimeri Europa®; UBEPOL-BR® rubbers, commercially available from UBE Industries, Inc.; BR 01, commercially available from Japan Synthetic Rubber Co., Ltd.; Neodene high-cis neodymium-catalyzed polybutadiene rubbers, such as Neodene BR 40, commercially available from Karbochem; TP-301 transpolyisoprene, commercially available from Kuraray Co., Ltd.; Vestenamer® polyoctenamer, commercially available from Evonik Industries; Butyl 065 and Butyl 288 butyl rubbers, commercially available from ExxonMobil Chemical Company; Butyl 301 and Butyl 101-3, commercially available from Lanxess Corporation; Bromobutyl 2224 and Chlorobutyl 1066 halobutyl rubbers, commercially available from ExxonMobil Chemical Company; Bromobutyl X2 and Chlorobutyl 1240 halobutyl rubbers, commercially available from Lanxess Corporation; BromoButyl 2255 butyl rubber, commercially available from Japan Synthetic Rubber Co., Ltd.; Vistalon® 404 and Vistalon® 706 ethylene propylene rubbers, commercially available from ExxonMobil Chemical Company; Dutral CO 058 ethylene propylene rubber, commercially available from Polimeri Europa; Nordel® IP NDR 5565 and Nordel® IP 3670 ethylene-propylene-diene rubbers, commercially available from The Dow Chemical Company; EPT1045 and EPT1045 ethylene-propylene-diene rubbers, commercially available from Mitsui Corporation; Buna SE 1721 TE styrene-butadiene rubbers, commercially available from Lanxess Corporation; Afpol 1500 and Afpol 552 styrene-

butadiene rubbers, commercially available from Karbochem; Nipol® DN407 and Nipol® 1041L acrylonitrile butadiene rubbers, commercially available from Zeon Chemicals, L.P.; Neoprene GRT and Neoprene AD30 poly-chloroprene rubbers; Vamac® ethylene acrylic elastomers, commercially available from E. I. du Pont de Nemours and Company; Hytemp® AR12 and AR214 alkyl acrylate rubbers, commercially available from Zeon Chemicals, L.P.; and Hypalon® chlorosulfonated polyethylene rubbers, commercially available from E. I. du Pont de Nemours and Company.

Suitable types and amounts of base rubber, initiator agent, coagent, filler, and additives are more fully described in, for example, U.S. Pat. Nos. 6,566,483, 6,695,718, 6,939,907, 7,041,721 and 7,138,460, the entire disclosures of which are hereby incorporated herein by reference. Particularly suitable diene rubber compositions are further disclosed, for example, in U.S. Patent Application Publication No. 2007/0093318, the entire disclosure of which is hereby incorporated herein by reference.

Suitable thermoplastic compositions include, but are not limited to, partially- and fully-neutralized ionomers, graft copolymers of ionomer and polyamide, and the following non-ionomeric polymers, including homopolymers and copolymers thereof, as well as their derivatives that are compatibilized with at least one grafted or copolymerized functional group, such as maleic anhydride, amine, epoxy, isocyanate, hydroxyl, sulfonate, phosphonate, and the like:

- (a) polyesters, particularly those modified with a compatibilizing group such as sulfonate or phosphonate, including modified poly(ethylene terephthalate), modified poly(butylene terephthalate), modified poly(propylene terephthalate), modified poly(trimethylene terephthalate), modified poly(ethylene naphthalene), including, but not limited to, those disclosed in U.S. Pat. Nos. 6,353,050, 6,274,298, and 6,001,930, the entire disclosures of which are hereby incorporated herein by reference;
- (b) polyamides, polyamide-ethers, and polyamide-esters, including, but not limited to, those disclosed in U.S. Pat. Nos. 6,187,864, 6,001,930, and 5,981,654, the entire disclosures of which are hereby incorporated herein by reference;
- (c) polyurethanes, polyureas, polyurethane-polyurea hybrids, and blends of two or more thereof, including, but not limited to, those disclosed in U.S. Pat. Nos. 5,334,673, 5,484,870, 6,506,851, 6,756,436, 6,835, 794, 6,867,279, 6,960,630, and 7,105,623, U.S. Patent Application Publication No. 2007/0117923, and U.S. Patent Application Ser. No. 60/401,047 and Ser. No. 13/613,095, the entire disclosures of which are hereby incorporated herein by reference;
- (d) fluoropolymers, including, but not limited to, those disclosed in U.S. Pat. Nos. 5,691,066, 6,747,110 and 7,009,002, the entire disclosures of which are hereby incorporated herein by reference;
- (e) non-ionomeric acid polymers, such as O/X- and O/X/Y-type copolymers, wherein O is an olefin (e.g., ethylene), X is a carboxylic acid such as acrylic, methacrylic, crotonic, maleic, fumaric, or itaconic acid, and Y is a softening comonomer such as vinyl esters of aliphatic carboxylic acids wherein the acid has from 2 to 10 carbons, alkyl ethers wherein the alkyl group has from 1 to 10 carbons, and alkyl alkylacrylates such as alkyl methacrylates wherein the alkyl group has from 1 to 10 carbons; including, but not limited to, those

disclosed in U.S. Pat. No. 6,872,774, the entire disclosure of which is hereby incorporated herein by reference;

- (f) metallocene-catalyzed polymers, including, but not limited to, those disclosed in U.S. Pat. Nos. 6,274,669, 5,919,862, 5,981,654, and 5,703,166, the entire disclosures of which are hereby incorporated herein by reference;
- (g) polystyrenes, such as poly(styrene-co-maleic anhydride), acrylonitrile-butadiene-styrene, poly(styrene sulfonate), polyethylene styrene;
- (h) polypropylenes, polyethylenes, propylene elastomers, ethylene elastomers, copolymers of propylene and ethylene, and blends of two or more thereof;
- (i) polyvinyl chlorides, and blends of two or more thereof;
- (j) polyvinyl acetates, preferably having less than about 9% of vinyl acetate by weight, and blends of two or more thereof;
- (k) polycarbonates, blends of polycarbonate/acrylonitrile-butadiene-styrene, blends of polycarbonate/polyurethane, blends of polycarbonate/polyester, and blends of two or more thereof;
- (l) polyvinyl alcohols, and blends of two or more thereof;
- (m) polyethers, such as polyarylene ethers, polyphenylene oxides, block copolymers of alkenyl aromatics with vinyl aromatics and poly(amic ester)s, and blends of two or more thereof;
- (n) polyimides, polyetherketones, polyamideimides, and blends of two or more thereof;
- (o) polycarbonate/polyester copolymers and blends of two or more thereof; and
- (p) combinations of any two or more of the above thermoplastic polymers.

Suitable ionomer compositions include partially neutralized ionomers and highly neutralized ionomers, including ionomers formed from blends of two or more partially neutralized ionomers, blends of two or more highly neutralized ionomers, and blends of one or more partially neutralized ionomers with one or more highly neutralized ionomers. Preferred ionomers are salts of O/X- and O/X/Y-type acid copolymers, wherein O is an  $\alpha$ -olefin, X is a  $C_3-C_8$   $\alpha,\beta$ -ethylenically unsaturated carboxylic acid, and Y is a softening monomer. O is preferably selected from ethylene and propylene. X is preferably selected from methacrylic acid, acrylic acid, ethacrylic acid, crotonic acid, and itaconic acid. Methacrylic acid and acrylic acid are particularly preferred. As used herein, "(meth) acrylic acid" means methacrylic acid and/or acrylic acid. Likewise, "(meth) acrylate" means methacrylate and/or acrylate. Y is preferably selected from (meth) acrylate and alkyl (meth) acrylates wherein the alkyl groups have from 1 to 8 carbon atoms, including, but not limited to, n-butyl (meth) acrylate, isobutyl (meth) acrylate, methyl (meth) acrylate, and ethyl (meth) acrylate. Particularly preferred O/X/Y-type copolymers are ethylene/(meth) acrylic acid/n-butyl (meth) acrylate, ethylene/(meth) acrylic acid/isobutyl (meth) acrylate, ethylene/(meth) acrylic acid/methyl (meth) acrylate, and ethylene/(meth) acrylic acid/ethyl (meth) acrylate. The acid is typically present in the acid copolymer in an amount of 6 wt % or greater, or 9 wt % or greater, or 10 wt % or greater, or 11 wt % or greater, or 15 wt % or greater, or 16 wt % or greater, or in an amount within a range having a lower limit of 1 or 4 or 6 or 8 or 10 or 11 or 12 or 15 wt % and an upper limit of 15 or 16 or 17 or 19 or 20 or 20.5 or 21 or 25 or 30 or 35 or 40 wt %, based on the total weight of the acid copolymer. The acid copolymer is at least partially neutralized with a cation source, optionally in the presence of a high

molecular weight organic acid, such as those disclosed in U.S. Pat. No. 6,756,436, the entire disclosure of which is hereby incorporated herein by reference. In a particular embodiment, less than 40% of the acid groups present in the composition are neutralized. In another particular embodiment, from 40% to 60% of the acid groups present in the composition are neutralized. In another particular embodiment, from 60% to 70% of the acid groups present in the composition are neutralized. In another embodiment, 60% to 80% of the acid groups present in the composition are neutralized. In another embodiment, from 80% to 100% of the acid groups present in the composition are neutralized. Suitable cation sources include, but are not limited to, metal ion sources, such as compounds of alkali metals, alkaline earth metals, transition metals, and rare earth elements; ammonium salts and monoamine salts; and combinations thereof. Preferred cation sources are compounds of magnesium, sodium, potassium, cesium, calcium, barium, manganese, copper, zinc, tin, lithium, and rare earth metals. In a particular embodiment, the ionomer composition includes a bimodal ionomer, for example, DuPont® AD1043 ionomers, and the ionomers disclosed in U.S. Patent Application Publication No. 2004/0220343 and U.S. Pat. Nos. 6,562,906, 6,762,246 and 7,273,903, the entire disclosures of which are hereby incorporated herein by reference. Suitable ionomers are further disclosed, for example, in U.S. Patent Application Publication Nos. 2005/0049367, 2005/0148725, 2005/0020741, 2004/0220343, and 2003/0130434, and U.S. Pat. Nos. 5,587,430, 5,691,418, 5,866,658, 6,100,321, 6,562,906, 6,653,382, 6,756,436, 6,777,472, 6,762,246, 6,815,480, 6,894,098, 6,919,393, 6,953,820, 6,994,638, 7,375,151, and 7,652,086, the entire disclosures of which are hereby incorporated herein by reference.

Also suitable are thermoplastic elastomers comprising a silicone ionomer, as disclosed, for example, in U.S. Pat. No. 8,329,156, the entire disclosure of which is hereby incorporated herein by reference.

The thermoplastic composition may contain additive(s) and/or filler(s) in an amount of 50 wt % or less, or 30 wt % or less, or 20 wt % or less, or 15 wt % or less, based on the total weight of the thermoplastic composition. Suitable additives and fillers include, but are not limited to, chemical blowing and foaming agents, optical brighteners, coloring agents, fluorescent agents, whitening agents, UV absorbers, light stabilizers, defoaming agents, processing aids, antioxidants, stabilizers, softening agents, fragrance components, plasticizers, impact modifiers,  $TiO_2$ , acid copolymer wax, surfactants, performance additives (e.g., A-C® performance additives, particularly A-C® low molecular weight ionomers and copolymers, A-C® oxidized polyethylenes, A-C® ethylene vinyl acetate waxes, and AClyn® low molecular weight ionomers, commercially available from Honeywell International Inc.), fatty acid amides (e.g., ethylene bis-stearamide and ethylene bis-oleamide), fatty acids and salts thereof (e.g., stearic acid, oleic acid, zinc stearate, magnesium stearate, zinc oleate, and magnesium oleate), oxides (e.g., zinc oxide, tin oxide, iron oxide, calcium oxide, aluminum oxide, titanium dioxide, magnesium oxide, and zirconium oxide), carbonates (e.g., calcium carbonate, zinc carbonate, barium carbonate, and magnesium carbonate), barium sulfate, zinc sulfate, tungsten, tungsten carbide, silica, lead silicate, clay, mica, talc, nano-filters, carbon black, glass flake, milled glass, flock, fibers, core material that is ground and recycled, and mixtures thereof. Suitable additives and fillers are more fully described in, for example, U.S. Patent Application Publication No. 2003/0225197, the entire disclosure of which is hereby incorporated herein by

reference. In a particular embodiment, the total amount of additive(s) and filler(s) present in the thermoplastic composition is 20 wt % or less, or 15 wt % or less, or 12 wt % or less, or 10 wt % or less, or 9 wt % or less, or 6 wt % or less, or 5 wt % or less, or 4 wt % or less, or 3 wt % or less, or within a range having a lower limit of 0 or 2 or 3 or 5 wt %, based on the total weight of the thermoset composition, and an upper limit of 9 or 10 or 12 or 15 or 20 wt %, based on the total weight of the thermoplastic composition. In a 10 particular aspect of this embodiment, the thermoplastic composition includes filler(s) selected from carbon black, micro- and nano-scale clays and organoclays, including (e.g., Cloisite® and Nanofil® nanoclays, commercially available from Southern Clay Products, Inc.; Nanomax® and Nanomer® nanoclays, commercially available from Nanocor, Inc., and Perkalite® nanoclays, commercially available from Akzo Nobel Polymer Chemicals), micro- and nano-scale talcs (e.g., Luzenac HAR® high aspect ratio talcs, commercially available from Luzenac America, Inc.), 15 glass (e.g., glass flake, milled glass, microglass, and glass fibers), micro- and nano-scale mica and mica-based pigments (e.g., Iridin® pearl luster pigments, commercially available from The Merck Group), and combinations thereof. Particularly suitable combinations of fillers include, 20 but are not limited to, micro-scale filler(s) combined with nano-scale filler(s), and organic filler(s) with inorganic filler(s).

The thermoplastic composition optionally includes one or more melt flow modifiers. Suitable melt flow modifiers 30 include materials which increase the melt flow of the composition, as measured using ASTM D-1238, condition E, at 190° C., using a 2160 gram weight. Examples of suitable melt flow modifiers include, but are not limited to, fatty acids and fatty acid salts, including, but not limited to, those disclosed in U.S. Pat. No. 5,306,760, the entire disclosure of which is hereby incorporated herein by reference; fatty amides and salts thereof; polyhydric alcohols, including, but not limited to, those disclosed in U.S. Pat. No. 7,365,128, and U.S. Patent Application Publication No. 2010/0099514, 35 the entire disclosures of which are hereby incorporated herein by reference; polylactic acids, including, but not limited to, those disclosed in U.S. Pat. No. 7,642,319, the entire disclosure of which is hereby incorporated herein by reference; and the modifiers disclosed in U.S. Patent Application Publication No. 2010/0099514 and 2009/0203469, the entire disclosures of which are hereby incorporated herein by reference. Flow enhancing additives also include, but are not limited to, montanic acids, esters of montanic acids and salts thereof, bis-stearyl ethylenediamine, monomers and polyalcohol esters such as pentaerythritol tetrastearate, zwitterionic compounds, and metallocene-catalyzed polyethylene and polypropylene wax, including maleic anhydride modified versions thereof, amide waxes and alkylene diamides such as bisstearamides. Particularly suitable fatty 40 amides include, but are not limited to, saturated fatty acid monoamides (e.g., lauramide, palmitamide, arachidamide behenamide, stearamide, and 12-hydroxy stearamide); unsaturated fatty acid monoamides (e.g., oleamide, erucamide, and ricinoleamide); N-substituted fatty acid amides (e.g., N-stearyl stearamide, N-behenyl behenamide, 45 N-stearyl behenamide, N-behenyl stearamide, N-oleyl oleamide, N-oleyl stearamide, N-stearyl oleamide, N-stearyl erucamide, erucyl erucamide, and erucyl stearamide, N-oleyl palmitamide, methylol amide (more preferably, methylol stearamide, methylol behenamide); saturated fatty acid bisamides (e.g., methylene bis-stearamide, ethylene bis-stearamide, ethylene bis-isostearamide, ethylene bis-hydrox-

ystearamide, ethylene bis-behenamide, hexamethylene bis-stearamide, hexamethylene bis-behenamide, hexamethylene bis-hydroxystearamide, N,N'-distearyl adipamide, and N,N'-distearyl sebacamide); unsaturated fatty acid bis-amides (e.g., ethylene bis-oleamide, hexamethylene bis-oleamide, N,N'-dioleyl adipamide, N,N'-dioleyl sebacamide); and saturated and unsaturated fatty acid tetra amides, stearyl erucamide, ethylene bis stearamide and ethylene bis oleamide. Suitable examples of commercially available fatty amides include, but are not limited to, Kemamide® fatty acids, such as Kemamide® B (behenamide/arachidamide), Kemamide® W40 (N,N'-ethylenebisstearamide), Kemamide® P181 (oleyl palmitamide), Kemamide® S (stearamide), Kemamide® U (oleamide), Kemamide® E (erucamide), Kemamide® 0 (oleamide), Kemamide® W45 (N,N'-ethylenebisstearamide), Kenamide® W20 (N,N'-ethylenebisoleamide), Kemamide® E180 (stearyl erucamide), Kemamide® E221 (erucyl erucamide), Kemamide® S180 (stearyl stearamide), Kemamide® 5221 (erucyl stearamide), commercially available from Chemtura Corporation; and Crodamide® fatty amides, such as Crodamide® OR (oleamide), Crodamide® ER (erucamide), Crodamide® SR (stearamide), Crodamide® BR (behenamide), Crodamide® 203 (oleyl palmitamide), and Crodamide® 212 (stearyl erucamide), commercially available from Croda Universal Ltd.

Non-limiting examples of suitable commercially available thermoplastics are Surlyn® ionomers and DuPont® HPF 1000 and HPF 2000 highly neutralized ionomers, commercially available from E. I. du Pont de Nemours and Company; Clarix® ionomers, commercially available from A. Schulman, Inc.; Iotek® ionomers, commercially available from ExxonMobil Chemical Company; Amplify® IO ionomers, commercially available from The Dow Chemical Company; Amplify® GR functional polymers and Amplify® TY functional polymers, commercially available from The Dow Chemical Company; Fusabond® functionalized polymers, including ethylene vinyl acetates, polyethylenes, metallocene-catalyzed polyethylenes, ethylene propylene rubbers, and polypropylenes, commercially available from E. I. du Pont de Nemours and Company; Exxelor® maleic anhydride grafted polymers, including high density polyethylene, polypropylene, semi-crystalline ethylene copolymer, amorphous ethylene copolymer, commercially available from ExxonMobil Chemical Company; ExxonMobil® PP series polypropylene impact copolymers, such as PP7032E3, PP7032KN, PP7033E3, PP7684KN, commercially available from ExxonMobil Chemical Company; Vistamaxx® propylene-based elastomers, commercially available from ExxonMobil Chemical Company; Vistalon® EPDM rubbers, commercially available from ExxonMobil Chemical Company; Exact® plastomers, commercially available from ExxonMobil Chemical Company; Santoprene® thermoplastic vulcanized elastomers, commercially available from ExxonMobil Chemical Company; Nucrel® acid copolymers, commercially available from E. I. du Pont de Nemours and Company; Escor® acid copolymers, commercially available from ExxonMobil Chemical Company; Primacor® acid copolymers, commercially available from The Dow Chemical Company; Kraton® styrenic block copolymers, commercially available from Kraton Performance Polymers Inc.; Septon® styrenic block copolymers, commercially available from Kuraray Co., Ltd.; Lotader® ethylene acrylate based polymers, commercially available from Arkema Corporation; Polybond® grafted polyethylenes and polypropylenes, commercially available from Chemtura Corporation; Royaltuf® chemically modified

EPDM, commercially available from Chemtura Corporation; Vestenamer® polyoctenamer, commercially available from Evonik Industries; Pebax® polyether and polyester amides, commercially available from Arkema Inc.; polyester-based thermoplastic elastomers, such as Hytrel® polyester elastomers, commercially available from E. I. du Pont de Nemours and Company, and Riteflex® polyester elastomers, commercially available from Ticona; Estane® thermoplastic polyurethanes, commercially available from The Lubrizol Corporation; Grivory® polyamides and Grilamid® polyamides, commercially available from EMS Grivory; Zytel® polyamide resins and Elvamide® nylon multipolymer resins, commercially available from E. I. du Pont de Nemours and Company; and Elvaloy® acrylate copolymer resins, commercially available from E. I. du Pont de Nemours and Company.

Golf balls of the present invention have at least one layer with a higher Shore C hardness and a lower Shore D hardness than that of another layer. For purposes of the present disclosure, such a layer having an atypical relative hardness relationship with at least one other layer of the ball (i.e., has either higher Shore C but a lower Shore D than another layer, or a higher Shore D but a lower Shore C than another layer) is referred to herein as an atypical hardness layer. In embodiments of the present invention wherein the ball comprises three or more layers, the golf ball has, in no particular order, a first atypical hardness layer, a second atypical hardness layer, and one or more additional layers, wherein each additional layer has a hardness that is:

- 30 (a) relatively harder on the Shore C and Shore D scales than the first and/or second atypical hardness layers;
- (b) relatively softer on the Shore C and Shore D scales than the first and/or second atypical hardness layers;
- (c) relatively harder on the Shore C scale and relatively softer on the Shore D scale than the first and/or second atypical hardness layers; and/or
- (d) relatively softer on the Shore C scale and relatively harder on the Shore D scale than the first and/or second atypical hardness layers.

40 For purposes of the present invention, a first layer has a higher Shore C hardness than a second layer if the Shore C hardness of the first layer is at least 1 Shore C unit greater than the Shore C hardness of the second layer. In a particular embodiment, the Shore C hardness of the first layer is at least 2 Shore C units, or at least 3 Shore C units, or at least 5 Shore C units, or at least 7 Shore C units, or at least 8 Shore C units, or at least 10 Shore C units, or at least 12 Shore C units, or at least 15 Shore C units, or at least 20 Shore C units greater than the Shore C hardness of the second layer.

45 For purposes of the present invention, a first layer has a higher Shore D hardness than a second layer if the Shore D hardness of the first layer is at least 1 Shore D unit greater than the Shore D hardness of the second layer. In a particular embodiment, the Shore D hardness of the first layer is at least 2 Shore D units, or at least 3 Shore D units, or at least 5 Shore D units, or at least 6 Shore D units, or at least 7 Shore D units, or at least 8 Shore D units, or at least 10 Shore D units, or at least 12 Shore D units greater than the Shore D hardness of the second layer.

50 In a particular embodiment, the golf ball includes a solid, single layer core and a single cover layer. In a particular aspect of this embodiment, the core has a higher Shore C hardness and a lower Shore D hardness than that of the cover, and, optionally, the core has a Shore C hardness of 86 or greater, or greater than 86, and a Shore D hardness of 60 or less, or less than 60, and/or the cover layer has a Shore C hardness of 86 or less, or less than 86 and a Shore D hardness

## 11

of 60 or greater, or greater than 60. In another particular aspect of this embodiment, the core has a lower Shore C hardness and a higher Shore D hardness than that of the cover, and, optionally, the core has a Shore C hardness of 88 or less, or less than 88, and a Shore D hardness of 60 or greater, or greater than 60, and/or the cover layer has a Shore C hardness of 88 or greater, or greater than 88, and a Shore D hardness of 60 or less, or less than 60.

In another particular embodiment, the golf ball includes a solid, single layer core, an inner cover layer, and an outer cover layer, wherein the inner cover layer is optionally formed from a composition comprising an ionomer, particularly an ionomer having an acid content of at least 16%, and a functionalized polyethylene. In a particular aspect of this embodiment, the core has a higher Shore C hardness and a lower Shore D hardness than the inner cover layer, and, optionally, the core has a Shore C hardness of 86 or greater, or greater than 86, and a Shore D hardness of 60 or less, or less than 60, and/or the inner cover layer has a Shore C hardness of 86 or less, or less than 86 and a Shore D hardness of 60 or greater, or greater than 60. In another particular aspect of this embodiment, the core has a lower Shore C hardness and a higher Shore D hardness than the inner cover layer, and, optionally, the core has a Shore C hardness of 88 or less, or less than 88, and a Shore D hardness of 60 or greater, or greater than 60, and/or the inner cover layer has a Shore C hardness of 88 or greater, or greater than 88, and a Shore D hardness of 60 or less, or less than 60.

In another particular embodiment, the golf ball includes an inner core layer, an outer core layer, an inner cover layer, and an outer cover layer, wherein the inner cover layer is optionally formed from a composition comprising an ionomer, particularly an ionomer having an acid content of at least 16%, and a functionalized polyethylene. In a particular aspect of this embodiment, the outer core layer has a higher Shore C hardness and a lower Shore D hardness than the inner cover layer, and, optionally, the outer core layer has a Shore C hardness of 86 or greater, or greater than 86, and a Shore D hardness of 60 or less, or less than 60, and/or the inner cover layer has a Shore C hardness of 86 or less, or less than 86 and a Shore D hardness of 60 or greater, or greater than 60. In another particular aspect of this embodiment, the outer core layer has a lower Shore C hardness and a higher Shore D hardness than the inner cover layer, and, optionally, the outer core layer has a Shore C hardness of 88 or less, or less than 88, and a Shore D hardness of 60 or greater, or greater than 60, and/or the inner cover layer has a Shore C hardness of 88 or greater, or greater than 88, and a Shore D hardness of 60 or less, or less than 60.

Golf balls of the present invention are typically finished by applying one or more finishing coats over the cover. For example, a primer and a topcoat may be applied. Either or both of the primer and topcoat compositions may be pigmented or clear. Several coats of clear or pigmented coatings may be applied.

Primer compositions are typically a solvent-borne or water-borne material, particularly selected from, but not limited to, polyurethanes, polyureas, acrylic polyurethanes, polyesters, polyester acrylics, and epoxies. In a particular embodiment, the primer composition is a two-part solvent-borne polyurethane comprising a resin component and an isocyanate component. In a particular aspect of this embodiment, the isocyanate component is present in an amount of from 31 parts to 35 parts, by weight per 100 parts of the resin component. In another particular aspect of this embodiment,

## 12

the resin component comprises from 50 to 58 wt % solids and the isocyanate component comprises from 46 to 53 wt % solids.

Topcoat compositions are typically a solvent-borne material particularly selected from, but not limited to, polyurethanes, polyureas, acrylic polyurethanes, polyesters, polyester acrylics, and epoxies. In a particular embodiment, the topcoat composition is a two-part solvent-borne polyurethane comprising a resin component and an isocyanate component. In a particular aspect of this embodiment, the isocyanate component is present in an amount of from 68 parts to 71 parts, by weight per 100 parts of the resin component. In another particular aspect of this embodiment, the resin component comprises from 46 to 52 wt % solids and the isocyanate component comprises from 46 to 53 wt % solids.

Primer and topcoat compositions optionally include additives including, but not limited to, pigments, tints, dyes, fillers, reaction enhancers or catalysts, crosslinking agents, optical brighteners, propylene carbonates, such as those disclosed in U.S. Pat. No. 5,840,788, which is incorporated in its entirety by reference herein, coloring agents, fluorescent agents, whitening agents, UV absorbers, hindered amine light stabilizers, defoaming agents, processing aids, mica, talc, nano-filters, wetting agents, solvents, and other conventional additives.

Non-limiting examples of suitable coatings are further disclosed, for example, in U.S. Pat. Nos. 5,409,233; 5,459,220; 5,494,291; 5,820,491; 5,669,831; 5,817,735; and 7,935,421, the entire disclosure of which are hereby incorporated herein by reference

In a particular embodiment, golf balls of the present invention comprise at least one coat of primer and at least one coat of topcoat. In a particular aspect of this embodiment, the primer is a solvent-borne composition and the topcoat is a solvent-borne composition.

Dimensions of golf ball components, i.e., thickness and diameter, may vary depending on the desired properties.

Golf ball cores of the present invention include single, dual, and multilayer cores, and preferably have an overall diameter within the range having a lower limit of 0.75 inches or 1 inch or 1.25 inches or 1.4 inches and an upper limit of 1.55 inches or 1.6 inches or 1.62 inches or 1.63 inches.

In a particular embodiment, the core is a solid, single layer having a diameter within a range having a lower limit of 0.750 or 1.00 or 1.10 or 1.15 or 1.20 or 1.25 or 1.30 or 1.40 or 1.50 or 1.53 or 1.55 inches and an upper limit of 1.55 or 1.60 or 1.62 or 1.63 or 1.65 inches. In a particular aspect of this embodiment, the core has a compression of 90 or less, or 80 or less, or 75 or less, or 70 or less, or a compression within a range having a lower limit of 50 or 55 or 60 or 65 and an upper limit of 65 or 70 or 75 or 80 or 90.

In another particular embodiment, the core comprises an inner core layer and an outer core layer, the inner core layer having a diameter within a range having a lower limit of 0.900 or 0.910 or 0.920 or 0.930 or 0.940 or 0.950 or 0.960 or 0.970 or 0.980 or 0.990 or 1.000 or 1.010 or 1.020 inches and an upper limit of 1.020 or 1.030 or 1.040 or 1.050 or 1.060 or 1.070 or 1.080 or 1.090 or 1.100 or 0.110 or 1.120 or 1.130 inches, and the outer core having a thickness within the range having a lower limit of 0.050 or 0.100 or 0.200 or 0.250 inches and an upper limit of 0.280 or 0.310 or 0.440 or 0.500 inches. In a particular aspect of this embodiment, the core has an overall dual core compression within a range having a lower limit of 60 or 70 or 80 or 85 and an upper limit of 85 or 90 or 95.

Golf ball covers of the present invention include single, dual, and multilayer covers, and preferably have an overall thickness within the range having a lower limit of 0.03 inches or 0.04 inches or 0.045 inches or 0.05 inches or 0.06 inches and an upper limit of 0.07 inches or 0.08 inches or 0.09 inches or 0.10 inches. Dual and multilayer covers have an inner cover layer and an outer cover layer, and multilayer covers additionally have at least one intermediate cover layer disposed between the inner cover layer and the outer cover layer. In a particular embodiment, the cover is a single layer having a thickness within a range having a lower limit of 0.020 or 0.025 or 0.030 inches and an upper limit of 0.030 or 0.040 or 0.045 or 0.050 or 0.070 or 0.100 or 0.120 or 0.150 or 0.350 or 0.400 or inches. In another particular embodiment, the cover comprises an inner cover layer and an outer cover layer, the inner cover having a thickness within a range having a lower limit of 0.020 or 0.025 or 0.030 or 0.035 inches and an upper limit of 0.035 or 0.040 or 0.045 or 0.050 or 0.100 inches, and the outer cover having a thickness within a range having a lower limit of 0.020 or 0.025 or 0.030 inches and an upper limit of 0.035 or 0.040 or 0.045 inches.

The present invention is not limited by any particular dimple pattern, dimple plan shape, dimple cross-sectional profile, or dimple size. Examples of suitable dimple patterns include, but are not limited to, phyllotaxis-based patterns; polyhedron-based patterns; and patterns based on multiple copies of one or more irregular domain(s) as disclosed in U.S. Pat. No. 8,029,388, the entire disclosure of which is hereby incorporated herein by reference; and particularly dimple patterns suitable for packing dimples on seamless golf balls. Non-limiting examples of suitable dimple patterns are further disclosed in U.S. Pat. Nos. 7,927,234, 7,887,439, 7,503,856, 7,258,632, 7,179,178, 6,969,327, 6,702,696, 6,699,143, 6,533,684, 6,338,684, 5,842,937, 5,562,552, 5,575,477, 5,957,787, 5,249,804, 5,060,953, 4,960,283, and 4,925,193, and U.S. Patent Application Publication Nos. 2006/0025245, 2011/0021292, 2011/0165968, and 2011/0183778, the entire disclosures of which are hereby incorporated herein by reference. Non-limiting examples of seamless golf balls and methods of producing such are further disclosed, for example, in U.S. Pat. Nos. 6,849,007 and 7,422,529, the entire disclosures of which are hereby incorporated herein by reference. In a particular embodiment, the dimple pattern is based on a spherically tiled tetrahedron. The dimples may have a variety of shapes and sizes including different depths and perimeters. In particular, the dimples may be concave hemispheres, or they may be triangular, square, hexagonal, catenary, polygonal or any other shape known to those skilled in the art. They may also have a cross-sectional profile based on any known dimple profile shape including, but not limited to, parabolic curves, ellipses, spherical curves, saucer-shapes, sine curves, truncated cones, flattened trapezoids, and catenary curves.

Golf balls of the present invention typically have a dimple count within a limit having a lower limit of 250 and an upper limit of 350 or 400 or 450 or 500. In a particular embodiment, the dimple count is 252 or 272 or 302 or 312 or 320 or 328 or 332 or 336 or 340 or 352 or 360 or 362 or 364 or 372 or 376 or 384 or 390 or 392 or 432.

For purposes of the present disclosure, the hardness of a thermoplastic composition or a thermoplastic golf ball layer is measured according to the following procedure. Hardness buttons of the composition (or layer) are compression molded under sufficient temperature and pressure for a sufficient amount of time to produce void- and defect-free

parts. The buttons are surface ground soon after the part reaches room temperature after demolding, to produce smooth, flat and parallel surfaces. The finished buttons are approximately 1.25 inches in diameter and at least 6 mm in thickness. The buttons are then aged for 10 days at 23° C. in a dessicator before testing. Hardness measurements are then made pursuant to ASTM D-2240 and/or JIS C (K6301 Type) using a calibrated, digital durometer, capable of reading to 0.1 hardness units and set to record the maximum hardness reading for each measurement. The digital durometer must be attached to, and its foot made parallel to, the base of an automatic stand having a travel speed of approximately 25 mm/sec.

For purposes of the present disclosure, the hardness of a thermoset composition refers to the surface hardness of a molded 1.55 inch diameter sphere of the composition. Similarly, the hardness of a thermoset golf ball layer refers to the surface hardness of a sphere, as measured on the golf ball layer. The surface hardness of a sphere is obtained from the average of a number of measurements taken from opposing hemispheres, taking care to avoid making measurements on the parting line of the sphere or on surface defects, such as holes or protrusions. Hardness measurements are made pursuant to ASTM D-2240 and JIS C (K6301 Type) using a calibrated, digital durometer, capable of reading to 0.1 hardness units and set to record the maximum hardness reading for each measurement. Because of the curved surface, care must be taken to insure that the sphere is centered under the durometer indentor before a surface hardness reading is obtained. The digital durometer must be attached to, and its foot made parallel to, the base of an automatic stand having a travel speed of approximately 25 mm/sec.

For purposes of the present disclosure, the compression of a sphere is determined according to a known procedure, using a digital Atti compression test device, wherein a piston is used to compress a sphere against a spring. Conversion from Atti compression to Riehle (cores), Riehle (balls), 100 kg deflection, 130-10 kg deflection or effective modulus can be carried out according to the formulas given in Jeff Dalton's *Compression by Any Other Name, Science and Golf IV, Proceedings of the World Scientific Congress of Golf* (Eric Thain ed., Routledge, 2002).

When numerical lower limits and numerical upper limits are set forth herein, it is contemplated that any combination of these values may be used.

All patents, publications, test procedures, and other references cited herein, including priority documents, are fully incorporated by reference to the extent such disclosure is not inconsistent with this invention and for all jurisdictions in which such incorporation is permitted.

While the illustrative embodiments of the invention have been described with particularity, it will be understood that various other modifications will be apparent to and can be readily made by those of ordinary skill in the art without departing from the spirit and scope of the invention. Accordingly, it is not intended that the scope of the claims appended hereto be limited to the examples and descriptions set forth herein, but rather that the claims be construed as encompassing all of the features of patentable novelty which reside in the present invention, including all features which would be treated as equivalents thereof by those of ordinary skill in the art to which the invention pertains.

**15****16**

What is claimed is:

1. A golf ball comprising:  
an inner core layer;  
an outer core layer formed from a rubber composition  
having a Shore C hardness of 86 or greater and a Shore 5  
D hardness of 60 or less, as measured on the surface of  
a molded 1.55 inch diameter sphere of the rubber  
composition;  
an inner cover layer formed from a thermoplastic com-  
position comprising an ionomer and a functionalized 10  
polyethylene, the thermoplastic composition having a  
Shore C hardness of less than 86 and a Shore D  
hardness of greater than 60, as measured on a hardness  
button formed from the thermoplastic composition; and  
an outer cover layer; 15  
wherein the Shore C hardness of the rubber composition  
is greater than the Shore C hardness of the thermoplas-  
tic composition; and  
wherein the Shore D hardness of the rubber composition  
is less than the Shore D hardness of the thermoplastic 20  
composition.

2. The golf ball of claim 1, wherein the ionomer has an  
acid level of 18% or greater.

\* \* \* \* \*